

Dec. 11, 1951

B. PILLER ET AL

2,577,915

METHOD FOR PRODUCING ARTIFICIAL FIBERS FROM HIGH MOLECULAR  
LINEAR POLYMERS OR POLYCONDENSATES RESPECTIVELY

Filed Sept. 21, 1949



INVENTORS:  
Bohumil Piller, Josef Zmatlik,  
Jan Pinkava, and Miroslav Starý  
BY

*Bohumil Piller*

## UNITED STATES PATENT OFFICE

2,577,915

METHOD FOR PRODUCING ARTIFICIAL  
FIBERS FROM HIGH MOLECULAR  
LINEAR POLYMERS OR POLYCONDEN-  
SATES RESPECTIVELY

Bohumil Piller, Varnsdorf, Josef Zmatlik, Brunn,  
Jan Pinkava, Prague, and Miroslav Starý,  
Zilina, Czechoslovakia, assignors to Zavody pre  
Chemicku Vyrobu, narodny podnik, Bratislava,  
and Elite, sdruzene tovarny puncoch, nardoní  
podnik, Varnsdorf, Czechoslovakia

Application September 21, 1949, Serial No. 116,992  
In Czechoslovakia September 21, 1948

6 Claims. (Cl. 18—54)

1

It is well known to produce strong fibers by spinning molten linear polymers into a cool, non-dissolving liquid medium, e. g. into water, or by cooling spun fibers a short time after having left the spinneret by bringing them into contact with a nondissolving liquid.

One device for said purpose forms object of co-pending patent application, Serial No. 96,593, now abandoned. It has been established however that polyamide or like fibers, which have not yet been oriented by cold drawing, became less strong when subjected for a long period of time to the influence of humidity. It is difficult to carry out the further treatment immediately at any time, and the said circumstance makes the quality of produced artificial fibers uneven.

It has been found that the disadvantage mentioned above can be avoided and the quality of produced fibers furthermore amended if fresh spun fibers, cooled by a nondissolving liquid medium are rapidly dried, e. g. by means of a concurrent stream of a dry, heated gas or air respectively or in any other way before subjecting them to the linear orientation. It is then possible to store them dry for any desired time in unoriented state before the cold drawing and subsequent treatment. This method is especially suitable for fibers having normal or a very small diameter where the cold drawing resistance never surpasses the tensile strength of unoriented fiber.

A preferred method of drying spun cooled fibers consists in drawing off the spun and water cooled fiber or fiber bundle respectively from the take up roller or rollers by means of an ejector with an extended diffusor, said ejector being driven by hot air or gas, streaming with such a speed, that the fiber bundle is easily separated from the surface of the last take up roller without being oriented by stretching.

The temperature of air or gas respectively introduced into the said ejector is preferably chosen so high, that the fiber is dried in a very short period of time, during which the fiber travels through the extended diffusor. The fiber bundle is then coiled up in usual way and subsequently treated by cold drawing, twisting etc., which operations may be carried out in any desired succession.

It has been established, that the fibers spun in the way described above have a substantially increased tensile strength in comparison with not dried ones or with such fibers, which have not been cooled by means of water in the neighbourhood of the spinneret, but have been stored for a long time in a room containing water vapors. This effect is due to the fact, that no

5 hygroscopic dilution of the low molecular components with a superfluous swelling of the polymerized fibrous mass takes place, which circumstance usually makes the complete orientation of molecules in one direction and in optimal mutual distance uneasy or impossible.

One embodiment of the present invention is shown in the following example in regard to the accompanying diagrammatical drawing.

- 10 The fiber bundle is led from the spinneret 1 over a grooved cylinder 2, concurrently with water running on its surface and then through a system of take up rollers 3 into the ejector 4. The inlet 5 is fed with nitrogen, preheated up to 200° C. under a starting pressure of 5 kg./cm.<sup>2</sup> so that the gas speed in the diffusor 6 reaches several hundreds of m./sec. and gives to the fiber bundle the tension necessary for separating it from the take up rollers 3 without stretching it up to the linear orientation. The fiber bundle is then coiled up or treated in any other unshown way. The tensile strength of fibers, e. g. of those from polymerized 6-caprolactam, increases by described treatment from 5 g. up to 6.8 g./den. The 25 drying may be carried out in any other suitable way, e. g. by using radiant heat and, if desired, by simultaneously using reduced pressure.

We claim:

1. A method for producing artificial filaments from molten high molecular fiber-forming materials which are capable of being oriented by cold drawing, comprising the steps of spinning said material; cooling the thus spun material by bringing a liquid into contact therewith; drying the thus cooled material; and cold drawing the thus dried material.

2. A method for producing artificial filaments from molten high molecular fiber-forming materials which are capable of being oriented by cold drawing, comprising the steps of spinning said material; cooling the thus spun material by bringing a non-solvent liquid into contact therewith; drying the thus cooled material; and cold drawing the thus dried material.

3. A method for producing artificial filaments from molten high molecular fiber-forming materials which are capable of being oriented by cold drawing, comprising the steps of spinning said material; cooling the thus spun material; drying the thus cooled material by means of an 45 ejector provided with a long diffusor and fed with a heated gaseous medium, said gaseous medium streaming with such a speed that the material is moved through the ejector without being linearly oriented; and cold drawing the thus dried material.

2

4. A method for producing artificial filaments from molten high molecular fiber-forming materials which are capable of being oriented by cold drawing, comprising the steps of spinning said material; cooling the thus spun material by bringing a liquid into contact therewith; drying the thus cooled material by means of an ejector provided with a long diffusor and fed with a heated gaseous medium, said gaseous-medium streaming with such a speed that the material is moved through the ejector without being linearly oriented; and cold drawing the thus dried material.

5. A method for producing artificial filaments from molten high molecular fiber-forming materials which are capable of being oriented by cold drawing, comprising the steps of spinning said material; cooling the thus spun material by bringing a non-solvent liquid into contact therewith; drying the thus cooled material by means of an ejector provided with a long diffusor and fed with a heated gaseous medium, said gaseous medium streaming with such a speed that the material is moved through the ejector without being linearly oriented; and cold drawing the thus dried material.

6. A method for producing artificial filaments

5  
10

4  
from molten high molecular fiber-forming materials which are capable of being oriented by cold drawing, comprising the steps of spinning said material; cooling the thus spun material by bringing a non-solvent liquid into contact therewith; passing the thus cooled material through a set of take up rollers; then drying the thus cooled material by means of an ejector provided with a long diffusor and fed with a heated gaseous medium, said gaseous medium streaming with such a speed that the material is moved through the ejector without being linearly oriented; and cold drawing the thus dried material.

15  
20

BOHUMIL PILLER.  
JOSEF ZMÄTLÍK.  
JAN PINKAVA.  
MIROSLAV STARÝ.

#### REFERENCES CITED

The following references are of record in the file of this patent:

#### UNITED STATES PATENTS

| Number    | Name    | Date         |
|-----------|---------|--------------|
| 2,354,744 | Dreyfus | Aug. 1, 1944 |
| 2,379,824 | Mummery | July 3, 1945 |